

## UNITED STATES PATENT OFFICE

2,588,640

## HYDROFUGATION OF TEXTILE MATERIALS

René Léon Lehmann, Paris, and Josef Lintner,  
 La Garenne Colombes, France, assignors to  
 Bozel-Maletra Societe Industrielle de Produits  
 Chimiques, Paris, France, a corporation of  
 France

No Drawing. Application November 4, 1948, Serial No. 58,370. In France April 26, 1948

13 Claims. (Cl. 260—67.6)

1

Some methods have already been proposed with a view to hydrophobing fabrics but, up to the present time none of them has made it possible to obtain a fibre which is both hydrophobic and strong, has a stable form and the hydrophobic effect of which is resisting to washing.

Now the applicants have found that it is possible to obtain in a simple manner both a strong unshrinkable fibre and, on the said fibre, a hydrophobic effect resisting to the known washing methods (such as the washing at ebullition with soap and sodium carbonate usually used for ordinary cotton, cellulose cotton and artificial silk or the chemical washing generally used for wool) by treating the textile fabrics or materials with stuffs obtained by condensing with a monovalent fatty alcohol containing a number of carbon atoms greater than 10, preferably from C<sub>15</sub> to C<sub>20</sub> in the presence of a weak acid, the products obtained according to the method described in the United States patent application No. 58,156 filed November 3, 1948 now Patent No. 2,574,114, issued November 6, 1951, for "Water-soluble condensation products for enhancing the qualities of textile materials" viz the products resulting from the condensation of an amide selected from the group consisting of urea, melamine and oxamide successively with glyoxal and with formaldehyde. In said copending application it is taught that by condensing an amide such as urea, melamine and oxamide in an acid medium with such an amount of glyoxal that it fixes only a portion, preferably not exceeding 50%, of the reactive nitrogen of the amide and by then treating the condensation products thus obtained in an alkaline medium with an amount of formaldehyde at least equal to the amount, stoichiometrically, to fix the remaining reactive nitrogen, it is very easy to obtain water soluble products containing in dry weight up to 45% of formaldehyde in combined form and having certain remarkable properties resulting from the presence of the glyoxal in the molecule; although the formaldehyde is thus combined in the molecule as a methylol group fixed on the nitrogen and although these said products are stable, non-volatile and not entrainable by aqueous vapor, nevertheless they still provide all chemical reactions of free formaldehyde without the risk of self-condensation into products having a higher molecular weight which would be difficultly soluble in water. In particular these methylols very easily form acetals with the hydroxyl groups of cellulose, even in the presence of water and even under the mere action of only slightly acid cata-

2

lysts, such as ammonium nitrate. This method of hydrophobing is distinguishable from the known methods by being easier to embody and by its remarkable effects: the reagents are used in an aqueous solution, which is a great advantage. On the other hand, the effects obtained are perfectly resisting not only to the known washing methods but also to most tinctorial baths, so that the treatment may be effected at any finishing stage of the textile materials. Since the treatment is effected in an only slightly acid medium, it does not cause any modification of the dye nor any damage to the fibre. Moreover the hydrophobic effect obtained does not affect in any manner the air permeability of the fabrics.

The preparation of the products intended for the treatment according to the invention may be effected by dissolving when heated and in an aqueous medium into a product prepared according to the method described in the above mentioned application, Serial No. 58,156, a small amount less than 7%, for example about 1%, of an emulsifying agent preferably a sulphonate of a fatty alcohol, after which the said solution is emulsified with such an amount of a monovalent fatty alcohol containing a number of carbon atoms greater than ten, preferably from C<sub>15</sub> to C<sub>20</sub>, for instance n-octadecyl alcohol that only a part of the methylol groups present may be etherified by the said alcohol, then, after acidification, the mixture is heated with reflux while vigorously stirring, until the reaction is completed. When cooling a white paste easily emulsifiable in distilled water is obtained.

The sulphonate used as an emulsifier may conveniently be that of the alcohol used for the condensation.

It is also possible to operate without any emulsifier. In this case a product prepared according to the above mentioned patent application is dissolved into solvents having a good affinity for water and a good dissolving power for fatty alcohols but which does not react with the methylol groups of the above products, e. g. N-methyl pyrrolidine, dimethyl formamide, methylol formamide, or other similar solvent, after which the water is first separated from the mixture by distillation, then the necessary amount of fatty alcohol is added and then, after acidification, the mixture is heated for a few hours. There is thus obtained nearly colourless products which dissolve in water to give a milky emulsion.

In order that the emulsions of the products thus obtained be stable even with hard water, it is advisable to add further the said products with

a small quantity of an emulsifier which may be prepared, for example by condensing n-octadecyl alcohol with about 20 moles of ethylene oxide. The amount of emulsifier to be added depends on the hardness of the used water and the harder the said water the greater the added amount of emulsifier. As an illustration, for a water having a hydrotimetric of 20-40 there will be added 0.5 to 1% in weight of emulsifier.

In order to obtain a maximum hydrophobic effect it is also advisable to add the condensation products with a moderately soft paraffin, having for example a melting point of about 40 to 50° C. a natural wax or a similar material easily soluble in fatty alcohols and producing a highly hydrophobic effect, the said substance, according to the quite unexpected findings of the applicant are then fixed upon the fibre and form thereon a combination which resists perfectly to the known washing methods.

The treatment of textile fabrics or materials with the products obtained according to the method described above is effected according to a mode of operation similar to that described in the patent application hereinbefore mentioned: the condensation products are set into a milky emulsion with water, then a catalyst such as ammonium nitrate is added and the textile product or fabric is impregnated with the said emulsion after which the product is wrung, dried and heated at a temperature preferably of about 110 to 120° C. for about 15 minutes.

The hydrophobic effect obtained on the textile products thus treated is materially stronger than that obtained on the same textile products by the known methods. The most remarkable fact is however that this hydrophobic effect as already mentioned above resists in a manner substantially absolute to the known washing method (washing at ebullition with soap sodium carbonate, chemical washing and the like), as well as to the tinctorial baths even to the aggressive baths used for the indigo and sulphur colouring matters.

When treating, in particular cellulose fibres, there is obtained simultaneously with the hydrophobic effect a reduction of the swelling power, an increase of the resistance to friction and an absolute form stability (unshrinkability).

The following example illustrates the invention but does not limit its scope in any manner.

#### Example

1.6 kg. urea is dissolved into 5.8 kg. of diluted aqueous glyoxal solution. The mixture is then acidified, for example by means of a small amount of high concentration hydrochloric acid and heated to ebullition. As soon as the glyoxal is combined, the mixture is allowed to cool down. The white precipitate of glyoxal-diurea is separated and then mixed with an alkaline aqueous solution of formaldehyde at 30% and the product thus obtained is then heated at ebullition until the formaldehyde is combined.

0.055 kg. of a moderately concentrated sulphonate obtained by a sulphonation of n-octadecyl alcohol with chlorosulphonic acid followed by a neutralization with caustic soda is dissolved while stirring at 70-80° C. into 5.3 kg. of an aqueous solution at about 50% of the condensation product prepared as described above. There is then added, while stirring, 0.54 kg. n-octadecyl alcohol and the whole is acidified with acetic acid. The mixture is then heated with reflux, while vigorously stirring until the

reaction is completed. Finally one dissolves into the mixture 0.75% by weight of the condensation product of about 20 moles of ethylene oxide with 1 mole of n-octadecyl-alcohol and paraffin having a melting point of 43 to 46° C. is finally also introduced. The still warm mixture is removed into an emulsifying apparatus and cooled down slowly therein to the room temperature. After cooling the paste should be homogeneous and its aspect should be similar with that of vaseline.

One then prepares in the cold, while stirring, with water having a hydrotimetric degree of 30, a milky emulsion containing per litre of water 50 g. of the above condensation product. 20 g. ammonium nitrate per litre are dissolved into the said emulsion, then the fabric to be treated is immersed into the solution while stirring for a few minutes. The fabric is then wrung until it remains on the fibre only a weight of solution equal to the weight of the original dry fabric. The fabric is then dried at 90° C. in a hot air current and finally the dry fabric is further heated for about 15 minutes at about 120° C.

Under the condition of this example, if the textile material to be treated was for example a regenerated cellulose fabric, after having been treated it is soft, agreeable and fleecy to the touch.

The hydrophobic effect obtained has been compared, before and after washing, with the effect obtained on the same fabric with the best hydrophobing methods known up to the present time:

Before the first washing, the hydrophobic effect obtained with the method according to the invention is about 9 to 10 times higher than the effect obtained with the best methods heretofore known. After five washings an ebullition with soap-sodium carbonate the hydrophobic effect obtained with the present method remains substantially unchanged, while the effect obtained with the best methods heretofore known drops after one single washing with soap-sodium carbonate at only 60° C., to  $\frac{1}{2}$  of its original value.

Even after 25 to 30 washings at ebullition, which however will probably never occur in the practice, the hydrophobic effect obtained with the present method is still about 50% of its original value; it thus remains still materially higher than the hydrophobic effect obtained with the best methods heretofore known.

In the above example the swelling power drops from the original value 100 to value 50 after the treatment; the said value of 50 is no more varied by the washings at ebullition with soap-sodium carbonate.

Similarly, the hydrophobic effect and the swelling power remain unchanged after extraction of the fabric with trichloro ethylene.

All above values are given to make the matter clear. In some cases, far more better results may be obtained.

What we claim is:

1. A method according to claim 7 in which the number of carbon atoms is comprised between 15 and 20.

2. A method according to claim 7 in which the condensation with the alcohol is effected without emulsifier but in the presence of a solvent having a good dissolving power for fatty alcohols and the product to be condensed with the alcohol but which does not react on the methylol groups of the product to be condensed with the alcohol.

3. A method of treating textile materials with a view to hydrophobing the same, consisting in impregnating the textile product to be treated with a solution of a condensation product according to claim 7 in the presence of a catalyst whereupon the said textile product is wrung, dried and heated.

4. A method according to claim 3 in which the catalyst is ammonium nitrate.

5. A method according to claim 3 in which the heating of the textile material is made at a temperature of 110 to 120° C. for about 15 minutes.

6. As new products of manufacture the hydrophobed textile products obtained by the method according to claim 3.

7. A method of manufacturing condensation products easily emulsifiable in water intended for enhancing the qualities of textile materials and more particularly for hydrophobing the same, consisting in heating in an acid medium a monovalent fatty alcohol containing at least 10 carbon atoms and not more than 20 carbon atoms, with a condensation product resulting from two steps: the first of which consists in the condensation of an amide selected from the group consisting of urea, melamine and oxamide, in an acid medium, with glyoxal; and the second step consisting in condensing the product thus obtained with formaldehyde in an alkaline medium, the amount of fatty alcohol used being such that only a portion of the methylol groups present is etherified.

8. A method of manufacturing condensation products easily emulsifiable in water intended for enhancing the qualities of textile materials and more particularly for hydrophobing the same, consisting in heating in an acid medium a monovalent fatty alcohol containing at least 10 carbon atoms and not more than 20 carbon atoms, with a condensation product resulting from two steps: the first of which consists in the condensation of an amide selected from the group consisting of urea, melamine and oxamide, in an acid medium, with such an amount of glyoxal that at most 50% of the hydrogen atoms of the amide groups present are substituted from the glyoxal; the second step consisting in condensing the product thus obtained with formaldehyde in an alkaline medium, the amount of fatty alcohol used being such that only a portion of the methylol groups present is etherified.

9. A method of manufacturing condensation products easily emulsifiable in water intended for enhancing the qualities of textile materials and more particularly for hydrophobing the same, consisting in heating in an acid medium a monovalent fatty alcohol containing at least 10 carbon atoms and not more than 20 carbon atoms, with a condensation product resulting from two steps: the first of which consists in the condensation of urea in an acid medium with glyoxal; and the second step consisting in condensing the product thus obtained with formaldehyde in an alkaline medium, the amount of fatty alcohol used being such that only a portion of the methylol groups present is etherified.

10. A method of manufacturing condensation products easily emulsifiable in water intended for enhancing the qualities of textile materials and more particularly for hydrophobing the same, consisting in heating in an acid medium a monovalent fatty alcohol containing at least 10 carbon atoms and not more than 20 carbon

atoms, with a condensation product resulting from two steps: the first of which consists in the condensation of urea in an acid medium with such an amount of glyoxal that at most 50% of the hydrogen atoms of the amide groups present are substituted from the glyoxal; the second step consisting in condensing the product thus obtained with formaldehyde in an alkaline medium, the amount of fatty alcohol used being such that only a portion of the methylol groups present is etherified.

11. A method of manufacturing condensation products easily emulsifiable in water intended for enhancing the qualities of textile materials and more particularly for hydrophobing the same, consisting in heating in an acid medium a monovalent fatty alcohol containing at least 10 carbon atoms and not more than 20 carbon atoms, with a condensation product resulting from two steps: the first of which consists in the condensation of melamine in an acid medium with glyoxal; and the second step consisting in condensing the product thus obtained with formaldehyde in an alkaline medium, the amount of fatty alcohol used being such that only a portion of the methylol groups present is etherified.

12. A method of manufacturing condensation products easily emulsifiable in water intended for enhancing the qualities of textile materials and more particularly for hydrophobing the same, consisting in heating in an acid medium a monovalent fatty alcohol containing at least 10 carbon atoms and not more than 20 carbon atoms, with a condensation product resulting from two steps: the first of which consists in the condensation of melamine in an acid medium with such an amount of glyoxal that at most 50% of the hydrogen atoms of the amide groups present are substituted from the glyoxal; the second step consisting in condensing the product thus obtained with formaldehyde in an alkaline medium, the amount of fatty alcohol used being such that only a portion of the methylol groups present is etherified.

13. As new products of manufacture, the condensation products obtained by heating in an acid medium a monovalent fatty alcohol containing at least 10 carbon atoms and not more than 20 carbon atoms, with a condensation product resulting from two steps: the first of which consists in the condensation of an amide selected from the group consisting of urea, melamine and oxamide, in an acid medium with glyoxal; and the second step consisting in condensing the product thus obtained with formaldehyde in an alkaline medium, the amount of fatty alcohol used being such that only a portion of the methylol groups present is etherified.

RENE LEON LEHMANN.  
JOSEF LINTNER.

#### REFERENCES CITED

The following references are of record in the file of this patent:

#### UNITED STATES PATENTS

|           |              |                |
|-----------|--------------|----------------|
| Number    | Name         | Date           |
| 2,427,504 | Morgan _____ | Sept. 16, 1947 |

#### FOREIGN PATENTS

|         |                     |               |
|---------|---------------------|---------------|
| Number  | Country             | Date          |
| 494,700 | Great Britain _____ | Oct. 13, 1938 |